

Patented Nov. 13, 1928.

1,691,882

# UNITED STATES PATENT OFFICE.

ROBERT W. HENRY, OF PORT ARTHUR, TEXAS, AND ELFORD D. STREETER, OF BAYONNE, NEW JERSEY, ASSIGNEES TO GULF REFINING COMPANY, OF PITTSBURGH, PENNSYLVANIA, A CORPORATION OF TEXAS.

## PROCESS OF PRODUCING THICKENED LUBRICATING OIL.

No Drawing.

Application filed March 24, 1926 Serial No. 97,116.

This invention relates to process of producing thickened lubricating oil; and it comprises a method of producing an improved lubricating oil of the type sometimes known as mineral castor oil and consisting of lubricating oil containing a dissolved or dispersed basic aluminum oleate or other basic aluminum soap wherein an aluminum soap of basic nature is produced by alkalizing a less basic 5 aluminum soap, and removing or reprecipitating the water soluble soap formed; all as 10 more fully hereinafter set forth and as claimed.

In the art what are known as mineral 15 castor oils or castor machine oils are extensively made by thickening mineral lubricating oil by an addition of a certain amount of aluminum oleate. This oleate is ordinarily a trioleate; that is, each atom of aluminum is 20 combined with three oleic acid groups. These trioleate preparations are generally made by direct precipitation of a solution of sodium oleate by an aluminum sulfate solution in the proper proportions. The precipitated aluminum soap so made is separated from the 25 mother liquor, which is a solution of sodium sulfate, washed, dried and added to the mineral oil to be thickened. The oleate goes into solution or dispersion and gives a great 30 increase in viscosity; the result wanted. In the usual types of mineral castor oil, however, this increase is neither regular nor constant. In adding a given quantity of oleate to a given oil, the exact increase in viscosity 35 is uncertain and the viscosity just after incorporation is by no means what it is after the thickened oil has been allowed to stand for a time and "age." There is always a marked drop in viscosity. In United States 40 Patent 1,550,608 is described a castor oil preparation free of the noted disadvantages; this preparation being made with basic oleates in lieu of the trioleate. Aluminum combines with oleic acid to form three different oleates 45 which may be represented, using the symbol R to represent the oleic acid group, as, respectively, the trioleate  $AlR_3$ , the dioleate  $AlR_2OH$  and the monoleate  $Al(OH)_2R$ . In the stated patent, it is pointed out that constant 50 preparations may be obtained by the use of basic oleates; oleates containing less oleic acid than the trioleate. The patent describes a ratio between R and Al of 1.7:1 or 1.8:1 as being most advantageous.

It is the purpose of the present invention 55 to provide a method whereby various mixtures of metallic oleates may be produced; the mixture, however, as a whole always being more basic than corresponds to the trioleate; mixtures, for example, of trioleate 60 and monoleate, of trioleate and dioleate, of di-oleate and monoleate, and of trioleate, dioleate, and monoleate. In the direct precipitation of a solution of sodium oleate by a solution of aluminum sulfate, which is the 65 usual way of making aluminum oleate, the tendency is to form a trioleate. In using the calculated quantities of aluminum sulfate and of soap for precipitation, the solution 70 generally becomes acid to phenol-phthalein before reaction is complete because of carrying down adsorbed sodium oleate. In practice therefore, it is the custom in precipitation to use an excess of aluminum sulfate or 75 alum and the result is the formation of trioleate. As stated, the trioleate is the substance generally used commercially in making thickened mineral oils or castors.

In the present invention, the purpose is to 80 make a basic oleate by a precipitation-hydrolysis method, using solutions of sodium soap, of caustic soda, and of aluminum sulfate. The composition of the final product depends upon the relative amounts of these 85 solutions taken, and upon the procedure followed. The general methods may be as follows. In one procedure, an aluminum trioleate is formed by the action of an excess of aluminum sulfate upon sodium soap solution, as just described, and then the requisite 90 amounts of caustic soda solution and aluminum sulfate solution, necessary to produce a basic oleate of predetermined basicity, are added to the aluminum trioleate portionwise and in alternation, the final addition being of aluminum sulfate. The mechanism of the reaction is hereinafter explained. In another method, caustic soda is added to aluminum trioleate in quantity sufficient to hydrolyze it to the aluminum monoleate, a predetermined portion of the solution of sodium soap formed by the hydrolysis is removed by 95 decantation, and aluminum sulfate is added to re-form aluminum trioleate from the sodium soap remaining. By each of the above 100 procedures, the final product contains principally aluminum monoleate and trioleate, with little or no dioleate present, even where

its average composition is that of a dioleate. This condition will be readily apparent to those skilled in the art in view of what has just been said. The reaction between sodium oleate or residual soap and aluminum sulfate produces aluminum trioleate, rather than the monoleate, which is already present, or the dioleate, which would result in the liberation of more caustic or more monoleate; 10 conditions which are contrary to the law of mass action. In still another procedure, the amount of caustic soda added to the aluminum trioleate is such as to give a mixture of aluminum mono- and di-oleates. Enough 15 caustic is added to effect hydrolysis, but not enough to replace two-thirds of the oleate present in combination with the aluminum. It may be assumed that, initially, all of the trioleate is converted to dioleate, and that 20 the excess caustic soda effects further hydrolysis to the monoleate to the extent that it is available. Substantially all of the sodium soap thus liberated in solution is then removed by decantation so that the final 25 product contains aluminum mono- and di-oleates with little or no trioleate. Generally, the stated operations are carried on in the presence of a body of the mineral oil to be used in forming the final castor; that is, the 30 work is done with emulsions rather than with simple solutions. The use of mineral oil and working in the emulsion form, however, while advantageous, is not necessary. Such mineral oil may be added at any stage of the 35 operation prior to the last addition of aluminum sulfate, but we usually add it in the beginning. Near the end of the last addition of "alum" the solution becomes acid, the emulsion breaks and the aluminum soap-oil 40 composition agglomerates into a pulp floating in a clear aqueous liquid containing sodium sulfate in solution.

In a general way, it may be said that the 45 trioleic soaps when admixed with ordinary lubricating oils of various grades give castors of relatively low viscosity, decreasing greatly on aging and sensitive to heat. Castors formed with dioleic soaps have a high initial viscosity, are adhesive, relatively insensitive to heat and of generally desirable properties, except that there is some decrease in viscosity on aging. On the other hand, castors formed from mineral oil and monoleic soaps, while having a high initial viscosity, become much more viscous upon aging and are relatively non-sticky and non-stringy. Mixtures of two or more of these aluminum soaps exhibit properties, when admixed with mineral oils which are the mean of the components. In making such mixed 55 aluminum soaps, a basic aluminum soap and a less basic aluminum soap may be made separately, and then mixed to form a product having the desired ratio of fatty acid to aluminum. On the whole, we find best for the

present purposes a mixture containing mainly aluminum monoleate and aluminum trioleate. The undesirable properties of the two balance each other out to a large extent. A 70 castor of suitable viscosity and desirable properties is obtained with a composite basic material corresponding to the formula



R, as before, indicating a molecule of oleic acid or any other fatty acid, but advantageously oleic acid or an unsaturated oily fat acid. The best results are obtained within the range  $\text{OH}_{1.5}\text{R}_{1.45}$  and  $\text{OH}_{1.45}\text{R}_{1.55}$ , which 80 expressions are, of course, arbitrary representations of the percentage composition of the mixture of two or more aluminum oleates of different basicities.

In practical embodiments of the present invention, while we can use a commercial soda soap as a starting material, we usually make a soap specially for the present purposes, preparing a neutral soda soap with the use of cottonseed oil or any other fatty oil. These oils, of course, contain glycerids of other fatty acids than oleic acid, but for the present purposes these acids are equivalent. The unsaturated acids of the oleic type are, however, better than the saturated. Corn oil works about as well as cottonseed oil. Stearic acid, oleostearine, cocoanut oil, and mixtures of these products with cottonseed oil are usually less satisfactory. Commercial oleic acid generally contains too much iron as an impurity, although it gives desirable products otherwise. In saponifying oil, the reaction is usually incomplete unless an excess of caustic soda is used. Thus the soap solution will usually contain free caustic. Any such excess alkali, we afterwards neutralize with 100 free fatty acid. It is best for our purposes to have a soap neutral to phenolphthalein when tested in alcohol. The neutral soap solution we usually emulsify with mineral oil of the same character as that to form the body 110 of the final castor. We generally employ a volume of mineral oil about twice that of the original cottonseed oil. The oil emulsifies readily, giving an "oil in water" emulsion; the water solution containing the soap. 115 In a practical application of the present invention, we start with about 750 pounds of cottonseed oil, and add 15° Baumé caustic soda solution in amount insufficient to saponify the oil. The mixture is stirred and blown with air for 3 or 4 hours and allowed to stand over night. The soap solution is then boiled and stirred or blown with steam for about an hour, after which small amounts of suitable fatty acid, such as a good grade of red oil, 120 are added until a test in alcoholic solution shows no color with phenolphthalein; indicating neutrality of soap. To this mixture is added 150 gallons of mineral oil and stirring is continued until the whole is emulsified and 130

is near the boiling point of the water solution. Operations at this range of temperature is most convenient and this temperature is maintained through the following stages 5 of the process. To the hot stirred mixture is next added an alum solution in amount slightly less than enough to precipitate all the sodium soap, say a solution containing 142 pounds of  $Al_2(SO_4)_3$ . The solution may 10 contain from 0.5 to 1 pound of "alum" per gallon and the addition should be spread over about an hour with a subsequent digestion to complete the reactions. If the aluminium sulfate contains an excess of acid this excess 15 should be neutralized by an addition of caustic soda. On the other hand, the aluminium sulfate solution may contain an excess of alumina, in which case a correspondingly less amount of caustic soda is used in the step 20 following. This addition of "alum" solution gives a soap approximating the trioleate; the trioleate containing adsorbed sodium oleate, and being suspended in slightly alkaline solution. In an alkaline medium, the pulp does 25 not agglomerate and the precipitates are in convenient physical form. In this embodiment of the invention, sodium soap is in excess and the solutions are alkaline up to the final addition of alum. We next add slowly 30 caustic soda solution in an amount equivalent to 66.5 pounds of  $NaOH$ . If the alum solution contains excess of alumina, as indicated above, an amount of  $NaOH$  corresponding to this basicity is deducted from the indicated 35 quantity of 66.5 pounds of  $NaOH$ . The caustic soda addition re-forms sodium oleate at the expense of the aluminium trioleate and produces aluminium monoleate. After the 40 caustic soda has been added, the stirring is continued for a time until a test (in alcoholic solution) shows no free caustic, or alkalinity. We next slowly add more alum solution thereby 45 reprecipitating the sodium oleate as aluminium trioleate which mixes with the basic aluminium soap already present forming a product somewhat less basic. An addition at this stage equivalent to about 82 pounds of  $Al_2(SO_4)_3$  works well. After the addition, stirring and heating are continued for a time 50 to complete the reactions. If the desired equivalent basicity of the aluminium soap is now attained, the precipitation may be completed by adding excess alum solution, and the pulp washed, dried, and diluted as here- 55 after explained. But, since a greater proportion of mono-aluminium soap in the mixture is usually desired, we next follow with another addition of caustic soda, this being added slowly, say, over a period of 1.5 to 2 hours. An addition of caustic equivalent to 60 about 38 pounds of  $NaOH$  is useful! After completion of the addition of caustic solution, digestion is continued until the mixture shows no free caustic. By this addition, 65 sodium oleate is again re-formed at the ex-

pense of the aluminium tri-oleate which is reduced to the monoleate. Finally, we complete the operation by adding alum solution to complete precipitation. Aluminium sulfate equivalent to about 140 pounds is added, 70 the addition extending over 2 hours. At this time, the aqueous portion of the batch will show a slightly acid reaction. The most desirable acidity is about pH 4.5.

In the operation just described in substance 75 there are a number of precipitations and re-precipitations, aluminium trioleate being converted into aluminium monoleate, and the sodium soap incidentally formed being reprecipitated as aluminium trioleate; the 80 amount of these actions decreasing as the process goes on. The final soaps resulting are largely a mixture of these two oleates. By modification in the quantities indicated, 85 dioleates in greater proportion can be produced. It is, of course, understood that the proportions are given in pounds and gallons as referring to a certain sized batch; one using 750 pounds of cottonseed oil.

The material produced after the last addition of aluminium sulfate is, as stated, a pulp 90 of thickened oil in a solution containing dissolved sodium sulfate and the glycerine of the original oil. When this product is formed, the stirrer is stopped and the separated aqueous liquor is drawn off. Water is then added to the pulp in the kettle and the 95 whole heated, using both open and closed steam. Usually a jacketed kettle is employed. The temperature is raised to near 100 the boiling point of water and the pulp and hot water stirred together for a short time, say, about 20 minutes, when the stirrer is stopped and the water removed. More water is added and the operation repeated, and so 105 on, until the wash water shows little or no sodium sulfate. Generally 5 or 6 washings are required. When washing is considered complete, the aqueous liquor is drained off 110 from the pulp as completely as possible and the pulp dried by heating and stirring until it is nearly clear in appearance. This portion of the operation requires considerable care to obtain the best results. To a considerable extent, the properties of the final 115 product depend upon drying to the right degree of hydration or dehydration. Complete dehydration gives an oil of viscosity no higher than the mineral oil; insufficient drying causes the soap to separate with production of cloudiness. Between these two extremes lies a very viscous pulp. When the pulp is dried to the desired extent, the heat is shut off and more mineral oil is added slowly with constant stirring, until a test 120 shows the desired viscosity of commercial mineral castor oil has been reached. With material made under the present invention, the viscosity shown in this test does not change materially on aging. 125

What we claim is:—

1. In preparing mineral castor oils containing basic aluminum soaps as thickeners, the process of preparing the thickener which comprises the steps of precipitating an aqueous solution of neutral fatty acid soap of an alkali with a sufficient quantity of a solution of an aluminum salt to convert said soap into a tri-acid soap of aluminum, then adding caustic alkali solution in amount sufficient to convert at least a portion of said tri-acid soap to a basic aluminum soap with production of neutral alkali soap, and then treating the resultant mixture with a solution of aluminum salt in amount sufficient to react with said alkali soap to form aluminum tri-acid soap. 69
2. In preparing mineral castor oils containing basic aluminum soaps as thickeners, the process of preparing the thickener which comprises the steps of mixing an aqueous solution of a neutral fatty soap of alkali with a sufficient quantity of a solution of an aluminum salt to convert said soap into tri-acid soap of aluminum and then adding caustic alkali solution in amount sufficient to convert at least a portion of said tri-acid soap to a basic aluminum soap. 70
3. In preparing mineral castor oils containing basic aluminum soaps as thickeners, the process of preparing the thickener which comprises the steps of mixing an aqueous solution of neutral fatty acid soda soap with a solution of aluminum sulfate in the proportions required to convert said soda soap into a tri-acid soap of aluminum, then adding caustic soda solution in amount sufficient to convert at least a portion of said tri-acid soap to a basic aluminum soap and then adding further aluminum sulfate solution to reprecipitate the sodium soap formed by the caustic soda. 73
4. In preparing mineral castor oils containing basic aluminum soaps the process which comprises mixing an aqueous emulsion of a fatty acid soap of an alkali and lubricating oil with a sufficient quantity of a solution of aluminum salt to convert the said soap into a tri-acid soap of aluminum, then adding caustic alkali solution in amount sufficient to convert at least a portion of said tri-acid soap to a basic aluminum soap with production of neutral alkali soap, then treating the resultant mixture with a solution of an aluminum salt in an amount sufficient to react with said alkali soap to form aluminum tri-acid

soap, washing the mixture, drying the washed mixture by heat until it becomes nearly clear in appearance, and adding sufficient further lubricating oil to give a mineral castor oil of the viscosity desired. 75

5. In preparing mineral castor oils containing basic aluminum soaps the process which comprises mixing an aqueous emulsion of a fatty acid soap of an alkali and lubricating oil with a sufficient quantity of a solution of aluminum salt to convert the said soap into a tri-acid soap of aluminum, then adding alkali solution sufficient to make the solution alkaline, then adding aluminum sulfate solution in amount sufficient to make the mixture become acid in reaction, washing the pulpy mass thus produced, drying by heat until it becomes nearly clear in appearance, and adding further lubricating oil to produce a mineral castor oil of the viscosity desired. 75

6. The process of preparing a thickener for mineral castor oils which comprises making a basic aluminum soap and a less basic aluminum soap, and mixing to form a product of the desired fatty acid to aluminum ratio. 80

7. In the manufacture of mineral castor oils containing basic aluminum soaps, the process which comprises emulsifying lubricating oil with an aqueous solution of neutral soap, precipitating by adding a solution of an aluminum salt, whereby a precipitate of tri-acid aluminum soap is formed, then adding sufficient caustic alkali solution to correspond to two-thirds of the fatty acid in said tri-acid aluminum soap, thereby forming a solution of alkali soap, adding a solution of an aluminum salt to re-produce aluminum soap at the expense of said alkali soap, thereby forming a mixture of soaps of different basicities, washing the mixture, drying the mixture by heat until it is nearly clear in appearance, and adding further lubricating oil to produce the viscosity desired. 85

In testimony whereof we have hereunto affixed our signatures at the places and on the dates indicated.

Signed at Port Arthur, in the county of Jefferson and State of Texas, this 18th day of March, 1926.

ROBERT W. HENRY.

Signed at Bayonne, in the county of Hudson and State of New Jersey, this 22nd of March, 1926.

ELFORD D. STREETER.

**CERTIFICATE OF CORRECTION.**

**Patent No. 1,691,882.**

**Granted November 13, 1928, to**

**ROBERT W. HENRY ET AL.**

**It is hereby certified that error appears in the printed specification of the above numbered patent requiring correction as follows: Page 1, line 64, after the words "sodium oleate" insert the word "soap"; line 80, after the word "basic" insert the word "metallic" and line 104, for the misspelled word "triolate" read "trioleate"; page 2, line 79, in the formula for "O H sub 1.5 R sub. 1.45" read "O H sub 1.55 R sub 1.45"; same page, line 119, for the word "insufficient" read "sufficient"; page 3, line 2, for the word "Operations" read "Operation"; same page, line 13, for the word "aluminium" read "aluminum"; and that the said Letters Patent should be read with these corrections therein that the same may conform to the record of the case in the Patent Office.**

**Signed and sealed this 8th day of January, A. D. 1929.**

**(Seal)**

**M. J. Moore,  
Acting Commissioner of Patents.**